

E. W. BEARDSLEY.

**PROCESS FOR HEATING AND SUBSEQUENTLY COOLING METAL ARTICLES.**  
APPLICATION FILED JULY 15, 1913. RENEWED APR. 14, 1916.

1,185,280.

Patented May 30, 1916.



Witnesses:

Chas. A. Pease  
John J. Grote

Inventor

*E.W. BEARDSLEY* Inventor

L. V. LEADBROOK  
By his Attorneys  
Bartlett, Franklin & Tolman

# UNITED STATES PATENT OFFICE.

EDWIN W. BEARDSLEY, OF CHESHIRE, CONNECTICUT, ASSIGNOR TO AMERICAN BRASS COMPANY, OF WATERBURY, CONNECTICUT, A CORPORATION OF CONNECTICUT.

## PROCESS FOR HEATING AND SUBSEQUENTLY COOLING METAL ARTICLES.

1,185,280.

Specification of Letters Patent.

Patented May 30, 1916.

Application filed July 15, 1913, Serial No. 779,103. Renewed April 14, 1916. Serial No. 91,264.

*To all whom it may concern:*

Be it known that I, EDWIN W. BEARDSLEY, a citizen of the United States, residing at Cheshire, New Haven county, Connecticut, 5 have invented certain new and useful Improvements in Processes for Heating and Subsequently Cooling Metal Articles, of which the following is a full, clear, and exact description.

10 My invention relates to a new and improved process of heating and subsequently cooling metal articles, and has for its object to provide for the heating and subsequent cooling of metals such as copper without 15 oxidation or discoloration of the same. It is particularly useful in annealing very fine copper wire.

The following is a description of an embodiment of my invention, reference being 20 had to the accompanying drawings, in which—

Figure 1 is a longitudinal section of an apparatus for carrying out my process, and Fig. 2 is a transverse section of the same on 25 the line  $x-x$ , Fig. 1.

Referring more particularly to the drawings, A is a furnace constructed of refractory materials in a common manner.

B is an oil or gas burner for supplying 30 fuel at the inner end of the combustion chamber and leading to the combustion chamber C from which the combustion gases pass through openings  $C_1$ ,  $C_2$  to the heating chamber D and from these are discharged 35 through outlet flue E.

F is a retort or muffle which may be made of metal or of refractory material and exposed either directly, as on the sides and top, or indirectly, as on the bottom, to the 40 heat of the furnace.

G is a gasket which makes air-tight the joint between the retort F and the cover or door H which is clamped against same by screws or clamps I.

45 J indicates coils of wire to be annealed.

K is a pipe leading to the interior of the retort at the top, open at  $K_1$  in the retort and connected by valve S with a source of steam L, preferably at low pressure, and by 50 valve R, with the atmosphere at or beyond M.

N is a pipe leading to the interior of the retort at the bottom, open at  $N_1$  in the retort and connected by valve Q with a source 55 of non-oxidizing gas such, for instance, as

illuminating gas, and by valve P, with the atmosphere at or beyond O.

In carrying out my process, the metal J to be heated is placed in the retort F and the door H is clamped in place. Valves Q 60 and R are closed. Valves P and S are opened, allowing steam from L to enter the retort through pipe K and opening  $K_1$  and drive the air out through opening  $N_1$  and outlet O. The retort F, and thus the metal 65 J, is then heated by the combustion of the fuel in chamber C and the hot gases as they travel through chamber D where a part of the combustion may take place. After the air has been driven out of retort F by the 70 steam, which must be accomplished before the retort F has been heated sufficiently to discolor the metal J, the outlet O may be closed by valve P, the steam inlet valve S being preferably left open to maintain the 75 steam in the retort at or above atmospheric pressure, which, for the sake of safety, should not be greatly exceeded, suitable reducing and safety valves being used if the steam is taken from an ordinary boiler. 80

When the metal has been heated sufficiently, the fuel supply is shut off and cold air is allowed to circulate through the chamber C, openings  $C_1$ , chamber D and flue E. Before the metal has cooled to the boiling point 85 of water, the steam supply valve S as well as the outlet valve P are closed. Gas supply valve Q and outlet valve R are then opened, allowing the gas to enter the retort at  $N_1$  and the steam to leave it at  $K_1$ . Gas 90 should be allowed to escape at  $K_1$  after the steam has been expelled, until all the moisture has been removed that can be carried out in that manner, when valve R may be closed. If the furnace is located in a building, outlet M should be continued to a suitable safe outlet when a combustible gas is used.

When the temperature of the metal has dropped to normal, or to such point as experience has proven suitable for the class 100 of work being done, gas supply valve Q should be closed and valves R and P should be opened to the atmosphere, thus allowing the gas to escape and air to enter and fill the retort. If outlet M is below the retort, 105 and the gas is lighter than air, air under pressure may be introduced through O or suction may be applied at M. When air has displaced the gas in the retort, the latter may be opened and the metal J removed. 110

It is obvious that the material heated may be other than copper and its alloys if similar advantage may be secured in similar manner. The heating may be for other purposes than 5 annealing. The steam used may be either saturated or superheated when introduced and the steam, particularly if it be superheated, may be the only vehicle for the transmission of heat to the interior of the retort. 10 The steam may be generated in the retort from water introduced therein. The moisture may be removed at a lower temperature than is described, by discharging a greater quantity of gas to carry out the moisture 15 condensed from the steam.

By the use of externally produced steam during the annealing process the amount of gas necessary is materially reduced.

What I claim is:

- 20 1. The process of treating oxidizable metal articles, which consists in heating them to the desired degree in a chamber filled with an atmosphere of steam from an external source, replacing said atmosphere by an atmosphere of non-oxidizing gas, and permitting the articles to cool to a non-oxidizing temperature while in the latter atmosphere. 25
2. The process of treating oxidizable metal articles, which consists in surrounding them 30 by an atmosphere of steam from an external source while contained in a chamber, applying heat externally to said chamber and thereby raising the temperature of the articles so surrounded to the desired degree,

replacing said atmosphere with an atmosphere of non-oxidizing gas, and permitting said chamber and the articles therein to cool to a non-oxidizing temperature. 35

3. The process of treating oxidizable metals, which consists in heating them while 40 in a chamber containing an atmosphere of steam from an external source, driving off said steam with a non-oxidizing gas, and cooling the articles to a non-oxidizing temperature while the chamber is filled with 45 such gas.

4. The process of treating oxidizable metals, which consists in heating them while 50 in a chamber containing an atmosphere of steam from an external source, applying external heat to said chamber, driving off said steam with a non-oxidizing gas, and cooling them and the chamber to a non-oxidizing temperature while the chamber is filled with 55 such gas.

5. The process of treating oxidizable metal articles, which consists in heating them in a chamber filled with an atmosphere of steam, cooling said chamber to a point above the boiling point of the moisture within said 60 chamber, replacing the atmosphere of steam thus cooled with an atmosphere of non-oxidizing gas, and cooling said chamber and its contents to a non-oxidizing temperature. 65

EDWIN W. BEARDSLEY.

Witnesses:

ARTHUR W. REDFERN,  
ALBERT B. BUTLER.